

Nov. 26, 1940.

P. M. CLARK ET AL

2,223,026

METAL CONTAINER

Filed Nov. 20, 1937



Percy M. Clark  
Charles B. Hemming  
BY

INVENTORS

Frank C. Shilberg ATTORNEY

## UNITED STATES PATENT OFFICE

2,223,026

## METAL CONTAINER

Percy M. Clark and Charles B. Hemming, Parlin,  
N. J., assignors to E. I. du Pont de Nemours &  
Company, Wilmington, Del., a corporation of  
Delaware

Application November 20, 1937, Serial No. 175,627

3 Claims. (Cl. 220—64)

This invention relates to a metal container for the packaging of food products or other perishable materials and more particularly to the production of an interiorly coated metal container, the coating of which is capable of protecting the metal from corrosion due to corrosive agents present in the packed material.

Metal containers interiorly coated with organic coatings of the oleoresinous type have been used for many years in the packaging of various foods, especially where the acid nature of the materials tends to attack the metal container and subsequently cause contamination of the food material through the absorption of the products formed by the corrosive action. It has been found in general that various classes of foodstuffs demand various types of protective coatings and much work has been done by the manufacturers of tin cans to provide coatings for each specific use.

A more recent development in the can industry has been the production of cans for the packaging of beer. It was found that the usual coatings were unsatisfactory and incapable of delivering the beer in a condition suitable for public consumption. Several factors appeared to cause this condition, among them, absorption of flavor-forming ingredients by the can coating, and the presence in the coating of soluble ingredients which when absorbed by the beer, markedly changed the taste thereof. In particular, it has been found that beer is especially subject to contamination and deterioration. Two types of coated containers have been developed which are being used commercially in large numbers at the present time. The first is a metal can with or without an organic primer coating and having a heavy wax coating as the top coat. The second type is a container with an organic priming coat and having a vinyl resin top coating.

Prior to and during the development of the above types of cans, considerable work was done by the industry in attempting to develop nitrocellulose lacquers for use as top coats and that these results were uniformly unsuccessful. Several reasons can be ascribed to these failures. First, failure to select suitable materials with which to modify the nitrocellulose. Second, failure to study the baking conditions and the solvent compositions required to give coatings free from traces of residual solvent which if present would cause serious contamination of the beer. Third, failure to work with modifiers purified to the extent absolutely necessary for

this work, and finally and more importantly, failure to recognize the necessity of reducing the permeability of the nitrocellulose film coating to water to a point much lower than commonly reached. Unmodified nitrocellulose coatings are much more permeable to water than is generally recognized, and when not suitably modified are inferior to the vinyl resin and wax coatings in commercial use.

The present invention is unique and commercially of interest in that the several defects of the nitrocellulose compositions and coating methods heretofore available for lining the interior of metal cans utilized in the packaging of beer, food products or other perishable materials, are eliminated.

An object of this invention is the provision of an interiorly coated container for the packaging of beer and the like, the coating of which is water-resistant, tough, flexible, adherent, insoluble, non-toxic, substantially impermeable to water and capable of protecting the metal from corrosion due to corrosive agents present in the packed material. Other objects will become apparent as the description of the invention proceeds.

These objects are accomplished by utilizing a specific type of modifier, consisting of a cyclohexyl derivative, in cellulose nitrate compositions, thus affording a lacquer which when coated on the interior of metal cans provides a convenient and commercially useful container.

In the practice of the invention, a priming coat is first applied to the metal surface before the application of the lacquer top coat. The qualifications for the primer are freedom from taste-contamination after baking, good adhesion to the metal surface and satisfactory coverage. The primer may be applied to flat sheets of black iron or tin or silver-plated metal by a roller coating machine at a prescribed coating weight which normally is about 4 milligrams of dry coating per square inch. The primer is baked at a temperature of about 380-425° F. for 10 to 15 minutes. Sections of the flat sheets are then formed into cylinders and the top coat applied to the interior by any suitable means, preferably by spraying. The can ends are usually coated with the lacquer before being formed. However, it is practicable to form the can ends directly following the baking of the primer and before the application of the lacquer top coat. In this case the lacquer would normally be applied by spraying.

*Example 1*

A suitable primer composition consists of a mixture of 5.5 parts of mineral spirits, 61.5 parts of hydrogenated naphtha of boiling range about 135 to 190° C., and 33 parts of a synthetic resin which is a reaction product of:

|                    | Per cent<br>by weight |
|--------------------|-----------------------|
| 10 Chinawood oil   | 12.3                  |
| Glycerine          | 18.8                  |
| Linseed oil        | 24.7                  |
| Phthalic anhydride | 44.2                  |
|                    | 100.0                 |
| 15                 |                       |

This resin is prepared by any of the methods well known and widely practiced in the art.

An alternative priming composition may consist of an oleoresinous varnish of conventional type, being prepared in the customary manner from drying oils and natural or synthetic gums. In general, it has been shown that oil lengths above 10 gallons in this type of base coat are liable to give a pronounced taste-contamination and the selection of the raw material for its preparation should be made with a view to minimizing its taste-producing characteristics.

Other commercially available priming compositions of similar constitution and properties may also be utilized as suitable base coats for the improved lacquer top coats hereinafter described.

The lacquer top coat is applied by spraying, roller-coating or dipping. It is then baked at a temperature not to exceed 300° F. for 8 to 10 minutes. The following examples are illustrative as representing the preferred embodiment of this invention:

*Example 2*

|                           | Per cent<br>by weight |
|---------------------------|-----------------------|
| 40 Cellulose nitrate      | 14.6                  |
| Dicyclohexyl phthalate    | 4.4                   |
| Ethyl alcohol (denatured) | 3.7                   |
| Ethyl acetate (absolute)  | 77.3                  |
|                           | 100.0                 |
| 45                        |                       |

*Example 3*

|                                 | Per cent<br>by weight |
|---------------------------------|-----------------------|
| 50 Cellulose nitrate            | 14.6                  |
| Dicyclohexyl hexahydrophthalate | 7.3                   |
| Ethyl alcohol (denatured)       | 3.1                   |
| Ethyl acetate (absolute)        | 50.0                  |
| Isopropyl acetate               | 24.4                  |
|                                 | 100.0                 |
| 55                              |                       |

*Example 4*

|                              | Per cent<br>by weight |
|------------------------------|-----------------------|
| 60 Cellulose nitrate         | 15.0                  |
| Dimethyl cyclohexylphthalate | 5.8                   |
| Ethyl alcohol (denatured)    | 4.0                   |
| Ethyl acetate                | 30.0                  |
| Methyl ethyl ketone          | 30.0                  |
| Isobutyl acetate             | 15.2                  |
|                              | 100.0                 |
| 65                           |                       |

The viscosity characteristic of the cellulose nitrate used in the above examples is about 3 seconds as determined in accordance with procedure outlined in A. S. T. M. specifications D-301-33, Formula B. Use of a lower viscosity material is possible but in general it leads to somewhat brittle films which do not permit satisfactory forming of the coated sheet metal. Use

of higher viscosity cellulose nitrate while preferable from the viewpoint of giving tougher films results in a lacquer having very low solids at the required spraying or applying viscosity. It is desirable to use the lowest viscosity cellulose nitrate commensurate with the flexibility desired of the film in order to produce the most economical finishes.

In Example 2, absolute ethyl acetate is used as the sole volatile solvent for the cellulose nitrate. The small amount of denatured ethyl alcohol is brought into the composition by the alcohol wet cellulose nitrate of commerce. This represents a volatile solvent vehicle which has been found to be the easiest to completely eliminate in the baking operation of the lacquer top coat. It is possible to employ a variety of other solvent combinations providing satisfactory baking conditions are set up. Medium boiling solvents such as isopropyl acetate, isobutyl acetate, normal butyl acetate, and in some instances volatile aliphatic hydrocarbon diluents can be used. Where the lacquers are to be applied by a roller coating machine it is required to have less volatile solvents than are necessary for spraying, but in every case practical tests must be made to determine the efficiency of the baking system and adjustment of the solvent composition. Minute traces of the volatile solvent remaining after the baking treatment will invariably contaminate the packed product.

Highly purified, odorless and tasteless dicyclohexyl phthalate was found to be outstandingly superior as a plasticizer in the cellulose nitrate compositions for the purpose indicated. However, dicyclohexyl hexahydrophthalate, dimethyl cyclohexyl phthalate, dicyclohexyl tartrate, tricyclohexyl citrate, cyclohexyl benzoyl benzoate and tricyclohexyl phosphate, and other cyclohexanol derivatives of carboxylic acids, when subjected to suitable purification treatments to render them odorless and tasteless are likewise suitable for use in the products of the present invention.

In addition to the normal function of the plasticizer which is the flexibilizing of the cellulose nitrate coating, this class of plasticizing materials greatly reduces the permeability of the lacquer film to the passage of water. The great majority of plasticizers of which dibutyl phthalate, castor oil and butyl oleate are representative, when added to nitrocellulose in increasing amounts at first cause a sharp lowering in permeability followed by an increase in permeability as the percentage of modifier is further increased. In the case of the previously mentioned cyclohexyl derivatives of carboxylic acids, it has been found that increasing the plasticizer content continuously decreases the permeability of the film at least up to about equal parts by weight of cellulose nitrate and plasticizer.

The superiority of the compositions of the present invention as regards liquid water permeability is clearly illustrated in the attached series of curves. The curves are derived by plotting the liquid water permeability of films prepared from the several compositions against plasticizer content and indicate the improved permeability factor which is obtained as the cyclohexanol derivative plasticizer content is increased to the desired range. The relatively poor permeability characteristic of compositions containing dibutyl phthalate and butyl oleate is also illustrated for comparison.

Numerical data from which the curves were

plotted was obtained as follows: A composition such as Example 2 is coated on both sides of a sheet of plain, transparent regenerated cellulose such as "Cellophane" to an overall thickness of .0004 inch of dry film. The coating is dried in a dry oven at 180-200° F. for one minute with circulating air. The dried film is then affixed across the top of a Petri dish, approximately 2½ inches in diameter by means of a molten adhesive composed of beeswax 85% and damar 15%, a quantity of water sufficient to completely cover the coated "Cellophane" when the dish is inverted, having been previously placed in the dish. The dish is accurately weighed, inverted and placed on a rack arranged so as to allow free circulation of air across the film. It is then placed in a thermostatically controlled oven at a temperature of 104° F. in which a relative humidity of less than 2% is maintained with forced air circulation, the air entering the oven having been dried by passing it through a series of bottles containing concentrated sulfuric acid. At the end of 18 hours the dish is removed from the oven and again accurately weighed. The results are expressed as grams of water lost per square meter per hour as utilized in plotting the curves on the accompanying graphs.

Minimum permeability is obtained when the cellulose nitrate-plasticizer ratios are within the range of 10-3 to 10-5 parts by weight. A satisfactory permeability reduction occurs with this new type of lacquer coat within the range of 10-3 to 10-10 parts by weight of cellulose nitrate to plasticizer.

In all instances this type of modifier greatly improves the adhesion and flexibility of the cellulose nitrate film and aids in the elimination of the last traces of solvent from the lacquer coating. It is tasteless, odorless, non-toxic and inert to hydrolysis.

This invention provides an interiorly coated metal container which is commercially satisfac-

tory for the packaging of beverages, particularly malt beverages, food products and other perishable materials. The new container meets the need in the industry for a can in which beer may be satisfactorily packed. It provides an interior surface coating which is poreless, substantially impervious to water, odorless and tasteless and capable of withstanding the deteriorating effect of beer and other beverages such as fruit juices and perishable foodstuffs which may also be safely packaged in the new containers.

It is apparent that many widely different embodiments of this invention may be made without departing from the spirit and scope thereof; and, therefore, it is not intended to be limited except as indicated in the appended claims.

We claim:

1. A metal container for beer and other beverages, foodstuffs and the like consisting of a tin plated metallic body interiorly coated with an alkyd resin priming coat and a top coat consisting of cellulose nitrate and a plasticizer compatible therewith, said plasticizer consisting of a cyclohexyl ester of a carboxylic acid in the ratio of between 10 parts by weight of cellulose nitrate to 10 parts of said plasticizer and 10 parts by weight of cellulose nitrate and 3 parts of said plasticizer.

2. A metal container for foodstuffs containing water, having a coating on at least the surface of the said metal container which is in contact with the foodstuff, said coating comprising in proportion 10 parts of nitrocellulose and from 3 to 10 parts of a highly purified cyclohexyl ester of a carboxylic acid as a plasticizer.

3. The container of claim 2 in which the plasticizer is selected from the group consisting of cyclohexyl and methyl cyclohexyl esters of the mono and dibasic carboxylic acids.

40

PERCY M. CLARK.  
CHARLES B. HEMMING.